

## UNITED STATES PATENT OFFICE

2,085,302

## METAL FOUNDING

Marvin W. Dundore, Beloit, Wis., assignor to  
 Beloit Iron Works, Beloit, Wis., a corporation  
 of Wisconsin

No Drawing. Application January 28, 1929,  
 Serial No. 335,750

6 Claims. (Cl. 22—188)

This invention relates to metal founding and has more particular reference to the manufacture of sand cores and molds. The present day commercial practice of casting ferrous and non-ferrous metals using sand molds and cores, is, and has been, handicapped by the varied and costly processes and operations required in freeing the castings of their cores and these difficulties are increased by reason of the many sizes and intricate shapes of the designs as well as by the varying requirements of workmanship in the finished casting. It is desirable to obtain cleaner and more accurate cast surfaces and shapes and to reduce the cleaning labor as much as possible. However, the attainment of these objects with cores of the prior art is beset with difficulties resulting from broken cores in handling after baking, cracked castings due to baked cores not contracting sufficiently as the metal contracts when cooling, core blows due to low permeability of the cores, crushed cores due to over-baking, dirty castings due to the surface skin of the core being washed to the surface of the casting, and distorted and strained castings due to the cores yielding slightly and temporarily arresting shrinkage. The faults of core binders now commonly used require close supervision on the part of the management and the laboratory, in order to minimize their effects upon the resultant product, the casting. There are, however, many other facts incidental to sand cores as now used and to their physical characteristics which are objectionable. For example, it is not infrequent that a casting, due to high shrinkage, cannot be prevented from cracking unless the cores are broken up as soon as the metal shows evidence of solidification. The uncovering of castings in order to partially or wholly remove the cores while the castings are still too hot to be handled is the cause of great discomfort as well as being attended with some little danger to the workmen who are subjected to flying hot sand and contact burns. Such premature removal of cores is also apt to be injurious to the castings be-

cause of accelerated cooling and consequent shrinkage cracks.

Another objection is that fusion of core sand takes place on the interior metal surfaces, which cannot be altogether removed by ordinary cleaning methods nor avoided by cautionary steps such as treating the surface of the cores with silica wash, graphite, or plumbago.

Consequently, fusion of sand to interior surfaces is apt to be harmful and apt to cause inextensible damage in cases where castings are used as conduits for steam and other liquids in machinery and systems of various cases.

Fusion of the molding sand also takes place at the interface between the mold and the metal and results in a rough outer surface and burned in portions of fused sand, which present an unsightly appearance and often materially interfere with the use of the casting unless removed. Considerable time and labor is involved in the cleaning of the outer surfaces.

My improvements in metal founding contemplate means for obviating these many difficulties in a simple and convenient manner whereby almost perfect castings of any size or shape may be obtained without resorting to the many cumbersome proceedings of the prior art.

I have also aimed to provide a new and improved sand core having the desired refractory properties whereby fusion of the core sand and "burning in" is effectively prevented.

A still further object of the invention is the provision of a method of preparing sand cores whereby considerable time is saved in the making thereof.

Another object is the provision of easy and effective means for treating sand molds whereby fusion of the mold sand with the surface of the casting is obviated and the use of plumbago or graphite is obviated.

The invention also contemplates the provision of a sand core which will permit the metal to freely contract on solidification offering no appreciable resistance thereto thereby avoiding internal strains and stresses in the casting and

deformation thereof either during solidification or after the casting has been put into use.

Another object is to provide a new and improved binding material for sand cores composed of a heat-plastic rubber isomer and suitable solvents.

One phase of my invention includes broadly the thorough mixing of dry core sand with a solution of a thermo-plastic rubber isomer, such, for example as the so-called Vulcalock cement, the forming of cores therefrom according to standard foundry practice, and the heat treatment thereof to convert the soft thermo-plastic materials into hard, high melting products and produce a hard, tough, refractory core.

I have discovered that when the so-called thermo-plastic rubber isomers or rubber derivatives are used as binders for the sand in making cores and treating the surface of molds and subjected to various treatments remarkably improved castings may be obtained therefrom. While little is generally known as to the chemical characteristics or the properties of this class of materials, they are formed by the treatment of undissolved rubber with agents having the general formula  $R-SO_2-X$  wherein R represents an organic radical or a hydroxy group and X represents a hydroxy group or chlorine, such reagents including sulfonic acid, organic sulfonic acids and organic sulfonyl chlorides or mixtures thereof. A mass of undissolved rubber is thoroughly masticated, for example, on an ordinary roller mill and the reagent is added directly to the rubber during working in the mill. When the reagent has been thoroughly dispersed throughout the rubber, the mixture is removed from the mill and heated. The product is then cooled and after removal from the oven is masticated on a warm mill to homogenize it and it may be washed free of remaining acid and other water soluble impurities during that process. Various other methods of reworking are also employed for homogenizing the product. Materials of various characteristics are obtained by varying the particular agent and the conditions of the process such as temperature, etc. Their preparation is described in some detail in U. S. Letters Patent Nos. 1,605,180 to Harry L. Fisher and 1,617,588 to William C. Geer, in the latter of which the materials are defined as "heat-plastic rubber isomers, a designation not wholly inapt for the reason that their main constituent has the same empirical formula as rubber and they possess a much higher degree of plasticity at moderately high temperatures than does rubber". The discoverers have given this class of materials the general name "thermoprene" using appropriate suffixes to indicate the various types. The only commercially obtainable material of this character so far as I am aware is the so-called "Vulcalock cement", having a base of the so called G. P. or gutta percha type, so called because of its resemblance to gutta percha. This material is formed through the use of pi-phenolsulfonic acid as a reagent.

In the preferred manner of practicing my invention I take a cement such as "Vulcalock" containing in the region of 18% of these heat-plastic rubber isomers and add thereto about an equal part by volume of gasoline or other cheap solvent with which the cement is miscible. I have found this proportion to be best suited for the purpose for practical reasons. More cement tends to make the resultant sand mixture too tacky and sticky while a lesser proportion produces a some-

what weaker core. I add this diluted cement in the ratio of about fifteen to one by volume to dry core sand of the kind ordinarily used in foundry operations. No particular care need be exercised in selecting the sand, one having the following analysis having been used with excellent results:

| Chemical analysis of sand used.      | Fineness | 10           |
|--------------------------------------|----------|--------------|
| SiO <sub>2</sub> .....               | 89.40    | Mesh 20..... |
| Al <sub>2</sub> O <sub>3</sub> ..... | 2.05     | 35.....      |
| Fe <sub>2</sub> O <sub>3</sub> ..... | 5.24     | 65.....      |
| CaO.....                             | 1.64     | 100.....     |
| MgO.....                             | .28      | 150.....     |
| K <sub>2</sub> O.....                | .59      | 200.....     |
| Na <sub>2</sub> O.....               | .40      | 270.....     |
|                                      |          | Pan.....     |
| Loss ignition.....                   |          | 0.32         |
| Moisture.....                        |          | Trace        |
| Clay.....                            |          | None         |

20

While any suitable means may be employed in mixing the cement into the sand, I have found it convenient to place the dry sand in a mixer having rotating blades and gradually add the requisite amount of the cement solution, running the mixer until the liquid cement has been thoroughly and uniformly incorporated into the sand. Each grain of sand should, by this time, be completely coated with a thin film of the adhesive cement. When properly mixed the mass has a certain sticky quality but will rub off the hands readily and will not adhere to the core box unless the same is waxed, for the diluted cement has a tendency to stick to a waxed box unless it has been thoroughly covered with some other coating.

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835

4840

4845

4850

4855

4860

4865

4870

4875

4880

4885

4890

4895

4900

4905

4910

4915

4920

4925

4930

4935

4940

4945

4950

4955

4960

4965

4970

4975

4980

4985

4990

4995

5000

5005

5010

5015

5020

5025

5030

5035

5040

5045

5050

5055

5060

5065

5070

5075

5080

5085

5090

5095

5100

5105

5110

5115

5120

5125

5130

5135

5140

5145

5150

5155

5160

5165

5170

5175

5180

5185

5190

5195

5200

5205

5210

5215

5220

5225

5230

5235

5240

5245

5250

5255

5260

5265

5270

5275

5280

5285

5290

5295

5300

5305

5310

5315

5320

5325

5330

5335

5340

5345

5350

5355

5360

5365

5370

5375

5380

5385

5390

5395

5400

5405

5410

5415</p

creases and the time required for heat treatment also increases, the time varying between a few minutes for relatively small cores and three to four hours for the largest cores. Large oil sand cores having a volume of 350 cubic inches of sand and requiring all night baking in a core oven, 425 degrees F., are prepared by my process in two hours, using the same oven and temperature.

Thus, by this method cores of all sizes, shapes, 10 and forms may be produced in a relatively short period of time having a hardness equal to or greater than baked oil or cereal bonded cores in all respects and useable in either green or dry sand molds.

15 The heat treated cores will withstand hard handling and abuse to a greater extent than oil sand cores and may be dropped without affecting the structure or shape to any appreciable degree. They do not shatter as do heat treated cores 20 and will not pulverize from handling in the core room.

Of great importance is the fact that the sand on the surface of the core does not fuse and "burn in" as is common in oil or cereal bonded 25 cores. The molten metal does not seem to affect the surface of these cores in the same manner as oil or cereal bonded cores, and, while I do not know the reason for this difference, I am led to believe that it is due to the great difference in 30 permeability of the two classes of cores as shown by the results of Standard A. F. A. tests, the excessive heat being conducted rapidly away from the core surface. Tests were run upon two simple oil sand cores which had been baked at 500° 35 F., for one hour. The permeabilities were 17 and 20. Tests were also made upon four cores prepared according to my invention and heat treated at 475° F., for twenty minutes. The permeabilities were 102, 120, 99 and 128, running from 40 five to six times greater than corresponding baked oil sand cores.

The fact that such "burning in" does not take place permits the casting of smooth internal surfaces which in most cases will require no further 45 treatment.

Again little care is required in heat treating my processed cores since fairly wide variations in temperature do not materially affect the result. However, with oil or cereal bonded cores 50 great care and considerable skill must be exercised in baking the cores to avoid overbaking and excessive temperatures and to produce a core of maximum strength.

The cores will not "wash" under the impact of 55 entering metal or the flow thereof over its surface due to the refractory and tough layer upon the surface of the heat treated core. Here again it is probable that due to the high permeability the heat is conducted rapidly away from the surface of the core preventing excessive local overheating. I have also found that the binding material of the heat treated cores is capable of withstanding considerably higher temperatures than the oil or cereal bonded cores without disintegration, which render them less susceptible to 60 "washing" with the metal.

Perhaps most important of all the thermo-plastic core does not obstruct the free contraction of the metal and is easily removed from the 70 casting, for as the metal contracts the core is gradually pushed from the casting as loose free flowing sand. While I do not know what occurs in the mold, other than that the sand is progressively released from bondage, I have formed a 75 theory as to the manner and reason of this oc-

currence which may or may not be true and I do not wish to restrict myself to the validity of the theory. I have found, however, that the core passes through a series of progressive changes. A core prepared as indicated above 5 having a volume of 91 cubic inches was placed in a gas heated furnace heated to an initial temperature of 450° F., and the temperature therein progressively raised. The following table will show the consecutive changes through which the 10 core passed:

| Core condition                                                                      | Time in minutes  | Temperature, °F. |
|-------------------------------------------------------------------------------------|------------------|------------------|
| Core placed in oven                                                                 | 0                | 525              |
| Core volatile ignited                                                               | 3                | 610              |
| Noticeable surface bond                                                             | 4                | 550              |
| Heavier encrustation, combustion gradually decreasing                               | 10               |                  |
| Decided crust $\frac{1}{8}$ " deep, combustion faded, interior core plastic or soft | 13               | 550              |
| Crust $\frac{1}{8}$ " deep                                                          | 20               | 550              |
| Started to raise temperature in order to quickly increase depth of crust            | 23 $\frac{1}{2}$ | 575              |
| Crust $\frac{1}{2}$ " deep                                                          | 25               | 610              |
| Core set very hard. Good for all practical purposes                                 | 35 $\frac{1}{2}$ | 1025             |
| Combustion of volatile resumed from interior core                                   | 36 $\frac{1}{2}$ | 1080             |
| Interior core soft                                                                  | 38 $\frac{1}{2}$ | 1100             |
| Spasmodic combustion volatile                                                       | 41               | 1160             |
| Core soft interior                                                                  | 42 $\frac{1}{2}$ | 1180             |
| Core still retaining full shape                                                     | 45               | 1200             |
| Very slight combustion                                                              | 45 $\frac{1}{2}$ |                  |
| Depth of exterior sand dry $\frac{1}{8}$ "                                          | 46 $\frac{1}{2}$ | 1220             |
| Depth of exterior sand dry $\frac{1}{8}$ "                                          | 49               | 1260             |
| Interior core still soft                                                            | 50               | 1280             |
| Core still retaining full shape                                                     | 51               |                  |
| Core still soft on interior                                                         | 53 $\frac{1}{2}$ |                  |
| Depth of exterior sand dry $\frac{1}{2}$ "                                          | 57               |                  |
| Depth of exterior sand dry $\frac{1}{2}$ "                                          | 59               | 1380             |
| No fracture in core surface. A gently re-ceding reversion to dry sand               | 65               | 1420             |
| Core readily disintegrated when disturbed                                           | 69 $\frac{1}{2}$ |                  |
| Certain resistance to disintegration still noticeable                               | 70 $\frac{1}{2}$ | 1500             |
| Core still erect                                                                    | 76               | 1600             |
| Certain resistance to complete disintegration                                       | 78               | 1620             |
| Reversion to full free flowing sand                                                 | 84 $\frac{1}{2}$ | 1680             |
|                                                                                     | 87 $\frac{1}{2}$ | 1700             |
|                                                                                     | 93               | 1720             |

It will be seen that decomposition of the binder does not begin until a temperature of approximately 1000° F. is reached. As the temperature increases the core progressively reverts to soft free flowing sand. I have assumed, therefore, that the action of the core under the heat of the molten metal in casting is somewhat similar, the core, because of the refractory properties of the binder, retaining its shape until the surface layer of metal has taken its initial set and then, as the excessive heat of the metal permeates the core, progressively breaking down, the surface of the core breaking down first, and liberating the sand to permit the contraction of the metal. Cores containing 114 cubic inches of my thermo-plastic bonded sand were immersed in a ladle of molten semi-steel as tapped from a cupola. Under this intense heat it required eight and one half minutes to make the transition from a thoroughly hardened core to entire loss of firm bond. It required twenty minutes for the core to revert to free flowing sand. Equivalent baked oil sand cores immersed in the ladle for twenty minutes revealed no sign of loss of bond and shape although heated half way through to a cherry red color. This clearly indicates the difference in the action of the two types of cores. The first retains its shape sufficiently long for casting purposes and then breaks down to permit the casting to contract, while the latter retains its shape and strength with persistency preventing the casting from contracting even though heated to a cherry red color.

Thus one result of my invention is a casting having no core strains from which the core is removed with ease and which has not been subjected to uneven cooling through the necessity of uncovering the hot casting to remove the core.

Another important characteristic of cores prepared according to my process is that they do not require venting as do other cores. There is very little smoke and no violent explosions such as accompany the use of oil and cereal bound cores. It is probable that this is due to the high permeability of the mass, and the fact that the decomposition of the ingredients does not take place until the core is sufficiently plastic to permit the escape of gases if formed. This completely eliminates the loss due to blow holes.

The cores because of their strength and refractoriness permit smaller cross-sections to be cast than is possible with other types of cores since there is no danger of fusion and the core is easily and cleanly removed. Nor do the heat treated cores require a "silica wash", "blacking", or any other surface wash in order to affect a smooth surface on the exterior of the core or increase its refractoriness. In this they are unlike all other cores as the surface of the core presents a smooth film having a high heat resistance.

It will have become evident that the cores after ramming can be made available for foundry use a great deal quicker than baked oil or cereal bonded cores of like weight and volume. By this process I produce a core fit for molding or casting purposes in 50 to 80% less time than is possible with a baked oil or cereal bonded core.

The cored surfaces do not have to be cleared of cores by or through the agency of core busting, sand blasting, hydraulic washing, pickling, chipping, tumbling, wire brushing, grinding, drilling, drifting or any other means for clearing the cores or removing burned-in or adhering sand since the cores do not fuse and thoroughly disintegrate under the casting heat.

Commercial castings have been made in brass, aluminum, bronze, gray iron, semi-steel and malleable iron using my improved cores. These castings have weighed up to and including twenty five hundred pounds and have been of plain and intricate design, utilizing plain slab cores, cylindrical shapes and pasted cores of intricate design and workmanship. All of these resulted in perfect commercial water and steam tested castings.

I have also found during the course of my investigation that when cores of small size are required the heat treatment may be dispensed with. In that case care must be taken in the selection of sand that it conform fairly closely with the analysis already given. In preparing cores of this kind the process is the same as previously outlined to the point where the core is heat treated except that the proportion of sand to diluted cement should be reduced to twelve to one or less in order to result in sufficient core strength. Instead of placing the cores in an oven they may be merely exposed to the air to permit the evaporation of the solvent from the outer portions thereof. They may be permitted to stand until they have attained sufficient hardness for use. Care must be taken to permit or cause sufficient movement of air over the cores to increase the rate of evaporation and prevent the accumulation of dangerous or explosive mixtures of solvent and air. Where, for example, only very small cores are used, or for some other reason heat treatment is not desired the small cores may

be prepared by simply drying them. This phase of the invention is limited, however, to small cores since in the larger ones the drying time becomes too great and sufficient core strength is not developed. When the larger sized cores are so prepared they are too flexible to be readily handled and the hard outer wall thereof is too soft to support the molten metal during casting.

Another factor which limits the size of the dried cores is the fact that vibrations and jars over the long drying period tends to shake the plastic mass down and develop cracks in the thinly formed crust thus distorting them, altering the shape and preventing their use with intricate designs. This may be partially overcome by careful rodding but in larger sizes the amount required becomes excessive.

Care must also be taken in choosing cores to be dried that the area thereof in contact with the supporting plate is small since these areas are very slow drying. The core, therefore, requires turning in order to permit the bottom to dry. If the core is too large or the bottom area too great a great deal of time is required before the crust becomes strong enough to support the core while it is being turned. The center and bottom thereof remains soft and when handled the fingers break through the crust or the core buckles and the soft center breaks out. For the same reason the cores cannot be placed in core driers to aid in retaining the form thereof when intricate shapes are desired, since covered areas will not dry with commercial speed. It is, therefore, necessary to heat treat such shapes.

Perhaps the most serious factor in limiting the size of the dried cores is that the larger cores will not withstand the molten metal since the skin is comparatively thin and there is a very large proportion of soft plastic sand beneath. The dried surface is plasticized at a low temperature and so becomes plastic with the first rush of metal, it, as well as the plastic sand beneath, being washed away by the impact of the incoming molten metal. The hydrostatic pressure of large volumes of metal also tends to deform the softened cores.

My invention further contemplates the use of the diluted thermo-plastic rubber isomers as a facing for sand molds. By the use of this liquid as a facing material the use of dry sand molds may generally be eliminated. Green sand molds, made from fresh, untreated sand, are cheap, but because of the moisture in the sand, fuse to and into the surface of the castings. In general practice this is avoided by preparing dry sand molds which involves heating the rammed molds to a temperature of 225 to 350° F., for about twelve hours. However, I have provided two ways in which all of the advantages of a dry sand mold and none of the disadvantages may be obtained from a treated green sand mold.

The green sand mold is prepared in the usual manner, after which the surface thereof is sprayed or otherwise treated with the diluted cement already described. Sufficient liquid should be applied to penetrate into the face to a depth of one fourth inch or less depending upon the weight of metal to be poured into the mold. The metal may be poured immediately after treating the mold if desired, and the resulting casting will have a smooth clean surface and will require no tumbling to remove the mold.

However, if desired, the procedure may be altered. In making the mold the patterns may first be covered with a layer of molding sand

which has been thoroughly mixed in the ratio of about fifteen to one with the diluted cement. The remainder of the mold may then be made from ordinary green sand and rammed up as is usual. The metal may be poured into the mold immediately if desired.

It will be evident that this phase of my invention is of considerable importance. All of the advantages of dry sand molds are obtained from 10 green sand molds yet the time required to produce them is 75% less. No baking is required and the mold is ready for use immediately after ramming. The costs of ovens, tracks, trucks, hoists, fuel, building space, and operators for handling the 15 same are eliminated.

While I have thus set out my invention in considerable detail it will be understood to be for purposes of illustration. I realize that numerous alterations and changes may be made without 20 materially departing from the spirit of the invention or the scope of the appended claims, in which—

I claim:

1. The method of making a core for metal casting consisting in mixing a quantity of sand 25 with a binder including a heat-plastic rubber isomer, forming a core of such mixture, and heating the same to a temperature sufficient to convert the isomer to a product melting at a higher temperature.

2. The method of making a core for metal casting consisting in mixing sand with a binder

including a heat-plastic rubber isomer, forming a core of such mixture, and heating the core to a temperature sufficient to convert at least a portion of the isomer to a product melting at a higher temperature.

3. The method of making a core for metal casting consisting in mixing a quantity of sand with a binder including a thermoprene of the G. P. type, forming a core of such mixture, and heat treating the same at a temperature sufficient to 10 convert the thermoprene to a product melting at a higher temperature.

4. The method of making a core for metal casting consisting in mixing a quantity of sand with a binder including a thermoprene of the 15 G. P. type, forming a core of such mixture, and heat treating the same at an elevated temperature between about 425 and 600° F.

5. The method of forming a core for metal casting consisting in mixing a quantity of sand with a 20 binder including a thermoprene, forming a core of such mixture, and heat treating the same between about 425 and 600° F. for a period of time dependent upon the size of the core.

6. The method of making a core for metal casting consisting in mixing about fifteen parts of sand with about one part of a binder including a solvent and a thermoprene, forming a core of such mixture, and heating the core to a temperature sufficient to convert the thermoplastic residue 30 to a product melting at a higher temperature.

MARVIN W. DUNDORE.